

May 8, 1923.

1,454,464

F. M. BECKET ET AL

CHROME IRON SHEET OR ARTICLE AND PROCESS OF MAKING SAME

Filed March 3, 1922



Inventors

Frederick M. Becket

Charles E. McQuigg

Bynes Townsend & Bissellstein,

Attorneys.

## UNITED STATES PATENT OFFICE.

FREDERICK M. BECKET, OF NEW YORK, AND CHARLES E. MCQUIGG, OF FLUSHING, NEW YORK, ASSIGNORS TO ELECTRO METALLURGICAL CO., A CORPORATION OF WEST VIRGINIA.

## CHROME-IRON SHEET OR ARTICLE AND PROCESS OF MAKING SAME.

Application filed March 3, 1922. Serial No. 540,885.

To all whom it may concern:

Be it known that we, FREDERICK M. BECKET and CHARLES E. MCQUIGG, citizens of the United States of America, residing at 5 565 Park Avenue, New York, and 356 Madison Ave., Flushing, L. I., in the counties of New York and Queens and State of New York, have invented certain new and useful Improvements in Chrome-Iron Sheets or 10 Articles and Processes of Making Same, of which the following is a specification.

This invention relates to ductile alloys of iron and chromium, and especially to such alloys in sheet form or in the form of articles embodying the sheet form of the alloy; and comprises a process whereby such physical properties may be imparted to the alloy as will enable its conversion into sheets or 15 sheet-metal articles of relatively high ductility. The invention comprises also the relatively ductile sheet or other article which may result from the practice of the said process, as well as the process involved in the manufacture of the said ductile sheet.

20 It is now well understood in this art that alloys comprising chromium and iron, associated with a small proportion of carbon (say not in excess of one percent) may be worked into sheet or other forms provided 25 the chromium content does not exceed a definite maximum which lies in the neighborhood of 16%. Such alloys are non-tarnishing in air at ordinary or somewhat higher temperatures, and have found many 30 applications in the arts. Such alloys are however incapable of withstanding the oxidizing action of air at extremely high temperatures, as from 1000° to 1100° C. Alloys containing substantially higher percentages 35 of chromium than the above, say approximately 20 per cent or upward, are substantially non-oxidizable in air at these high temperature ranges, as already disclosed in a prior Patent No. 1,245,552 patented Nov.

40 6, 1917, to F. M. Becket; but such alloys have never to our knowledge been successfully rolled into sheet of commercial grade and quality; although they have been successfully forged into a great variety of articles. In this connection it should be clearly 45 understood that an alloy which is capable of being rolled into sheet can also, as a rule, be hot-pressed or drawn at least into rela-

tively shallow forms; and conversely an alloy which can be drawn is capable of being 55 rolled: but many alloys can be forged or swaged, although they can neither be rolled nor drawn. For example in the prior patent to Becket, above mentioned, referring to alloys containing 20-35% of chromium associated with say 1.5-3.0% of carbon it is 60 stated:

"Alloys within the limits above specified possess a strongly marked fibrous structure. They can be forged and machined, although 65 with difficulty as compared with ordinary steel. They can be annealed and also tempered, and in general are responsive to heat treatment, although to a materially less degree than ordinary high-carbon steels."

70 It is obvious that great commercial and technical advantages would follow if iron-chromium alloys lying within that we will term the non-oxidizable range, meaning thereby substantially non-oxidizable in air 75 at all temperatures up to 1000° or 1100° C., could be transformed into non-brittle sheets and into the numerous commercial articles which might with advantage include or embody the metal in sheet form: and it is a 80 primary object of the present invention to provide a process by which this result can be accomplished in a practical and commercial manner.

85 In the practice of our process in its preferred embodiment we prepare a non-oxidizing alloy containing upward of 20 per cent of chromium, associated with some carbon, the balance being principally iron. Relatively small proportions of other metals, 90 such as manganese, silicon, copper or the like may of course be present, provided they are not in sufficient proportion to interfere with those properties of the alloy which are essential to our present purposes. We prefer a carbon-content below 0.5%; and in general, the lower the carbon content the more readily and cheaply the alloy is rolled or drawn. But our invention is not restricted to such low carbon ranges, as we have successfully rolled alloys containing in excess 95 of 1 per cent of carbon. High carbon content is however usually regarded as undesirable, not only on account of the increased difficulty and expense of rolling as mentioned above, but because the higher carbon 100 105

alloys are increasingly liable to harden to an undesirable extent when quenched or otherwise quickly cooled.

Our preferred rolling temperature is between 800° and 1000° C. The higher the carbon content, the higher the preferred rolling temperature; but in no case should a temperature of 1100° C. be greatly exceeded. To insure the best results the first passes should be of relatively light draft, which may be increased as the rolling progresses. In this respect these alloys, particularly those of high carbon or chromium content differ sharply from steel, the difference being in all probability associated with the relatively poor welding properties of the alloy, with the attendant risk of breaking down the inherently weak large crystals before the refining has taken place.

We have discovered that in order to impart to the alloy such ductility as will permit us to make a finished sheet of satisfactory ductility and physical properties, it is essential first, that the sheet should be cooled from a temperature not lower than about 600° C. and preferably 800 or 900° C.; and second that the cooling from about 600° to about 400° C. should be rapid. The rate of cooling below about 400° C. or above about 600° C. seems to be without substantial effect on the quality of the alloy. If however the sheet is permitted to cool slowly through the range 600°-400° C. it is liable to become so embrittled as to be non-usable for most commercial purposes. It will of course be understood that the upper and lower limits of this embrittling temperature range are only approximately expressed above, since different alloy compositions do not act identically in this respect; but good results can be assured by rapid cooling through the range specified. Sufficiently rapid cooling can be secured in the case of thin sheets by an airblast; but with thicker sheets the best practice involves quenching from a temperature not less than 600° C.

There are two principal ways in which ductile sheets may be prepared in accordance with our process. According to the first way, the rolling with or without reheating between passes is carried through in such manner that the finishing temperature will lie above 600° C., in which case the sheets can be quickly cooled through the embrittling range of 600°-400° C., with resulting direct production of commercially ductile sheets. This is however often difficult of accomplishment, particularly when the sheets are relatively thin; and in such case substantially the same result can be attained by reheating the finished sheets to a point above 600° C. and preferably to or above 800° C. and cooling them rapidly through the above mentioned embrittling range. For the best results the total time during which the metal

is passing through the range from 600°-400° C. should not much exceed one minute; and is preferably as much less than this as is practicable under the particular circumstances.

By application of the above principles we have been able to prepare chrome iron sheets of a degree of ductility adequate for commercial purposes from a wide range of non-oxidizable alloys, varying from a minimum chromium content approximating 20%, to a maximum of about 60%; and it is probable that the principles are applicable even above this latter figure. The property of "ductility" as the term is used in this specification may be indicated or measured in various ways, as for example by the so-called "bend test"; or, and preferably, by the Erichsen value. According to this last-mentioned test a rounded point of standard radius of curvature is pressed into the surface of a marginally supported sheet of the metal to be tested to a depth at which the initial fracture occurs, the depth of penetration expressed in millimeters being the Erichsen value. A typical chrome-iron sheet, prepared in accordance with this invention from alloys within the non-oxidizable range, will give an Erichsen value not less than 5, and up to 7 or higher, for a 20 gauge sheet.

For a given alloy composition and thickness of sheet, providing in all cases that the metal has been properly carried through the embrittling range of about 600°-400° C., the Erichsen value appears to depend directly upon the temperature from which the sheet has been cooled. This relation is graphically shown in the accompanying drawing, in which the figure is a curve expressing in millimeters the Erichsen values of a No. 20 gauge sheet (.020 inch in thickness) rolled from an alloy of the following composition:

|           | Per cent. | 110 |
|-----------|-----------|-----|
| Chromium  | 28.50     |     |
| Carbon    | 0.33      |     |
| Silicon   | 0.79      |     |
| Manganese | 0.28      |     |

the balance substantially all iron; the sheet being cooled from various temperatures as indicated on the drawing. As will be noted, in this particular case the values rise from a minimum of 2 in the sheet cooled from a temperature lying within the embrittling range of 400°-600° C., to a maximum of 7 at our preferred rolling or reheating range of 800°-1000° C.; and again tend to fall as this temperature is exceeded. It will be understood by those familiar with this art, that a specific Erichsen number is valid only for a definite thickness of sheet; but for any given metal the values for varying sheet-thickness follow a known type of curve, so that the corresponding values for other sheet-thicknesses can as a rule be approximated 130

with sufficient accuracy for commercial purposes. For this reason the Erichsen value for a given sheet thickness will serve as an index of the quality of ductility in the metal. So far as we are aware, we are the first to prepare chrome iron alloys within the non-oxidizable range, that is to say containing more than about 20% of chromium, in the form of non-brittle sheets; and we regard such sheets, or articles made from or embodying the same, as a part of our invention. The term "sheet" is employed herein in its broad sense, to include those heavier products which are sometimes designated in the trade as "plate."

It has heretofore been believed that the workability of iron-chromium alloys decreases quite regularly with increasing chromium content. Our investigations have disclosed however that such is by no means the case, and that at least over a very considerable range of carbon content, alloys containing upward of about 40% of chromium are decidedly more easily worked than are alloys of similar carbon content but containing around 30-35% of chromium. As an example of this we have been able readily to roll into a commercial grade of sheet alloys containing in addition to iron:

|    |                |       |       |
|----|----------------|-------|-------|
| 30 | Chromium-----  | 52.38 | 52.20 |
|    | Carbon-----    | 2.18  | 1.40  |
|    | Silicon-----   | 1.00  | 0.75  |
|    | Manganese----- | 1.36  | 0.66  |

35 Such alloys not only possess the characteristic of resistance to oxidation at high temperature ranges, but possess qualities of resistance to many chemical reagents which fit them particularly for such specific uses as 40 dental spatulas, surgical instruments and the like.

We claim:

1. Process of making chrome-iron sheets or articles of relatively high ductility, comprising mechanically reducing the metal to sheet by rolling, drawing or equivalent steps; and subsequently rapidly cooling the heated sheet through the temperature range 600°-400° C.
- 50 2. Process according to claim 1 in which the rolled or drawn sheet is reheated, and then rapidly cooled through the temperature range 600°-400° C.

3. A non-brittle sheet or article having the characteristics and structure of rolled or drawn iron-chromium alloy; presenting surfaces substantially non-oxidizable in air up to at least 1000° C.; and containing upward of 20% chromium, the balance principally iron.

4. A non-brittle sheet or article having the characteristics and structure of rolled or drawn iron-chromium alloy; presenting surfaces substantially non-oxidizable in air up to at least 1000° C.; and containing upward of 40% chromium, the balance principally iron.

5. A sheet or article having the characteristics of rolled or drawn iron-chromium alloy; presenting surfaces substantially non-oxidizable in air up to at least 1000° C.; and containing upward of 20% chromium, the balance principally iron; said article having substantially higher ductility as measured by the Erichsen value than a non-heat-treated sheet of the same thickness and composition.

6. A sheet or article having the characteristics and structure of rolled or drawn iron-chromium alloy; presenting surfaces substantially non-oxidizable in air up to at least 1000° C.; and containing upward of 20% chromium, the balance principally iron; said article having an Erichsen value of not less than five millimeters in a thickness corresponding to that of a 20 gauge sheet.

7. A rolled iron-chromium alloy containing upward of 40% chromium, and upward of 1.5% carbon, the balance principally iron.

8. A rolled iron-chromium alloy containing upward of 40% chromium.

9. A non-brittle heat-treated sheet or article having the characteristics and structure of rolled or drawn iron-chromium alloy, and containing upward of 40% chromium, the balance principally iron.

10. Process of heat-treating chrome-iron alloys to impart ductility thereto, comprising rapidly cooling the heated alloy through the temperature range 600°-400° C.

In testimony whereof, we affix our signatures.

FREDERICK M. BECKET.  
CHARLES E. MoQUIGG.